

## UNITED STATES PATENT OFFICE

HAROLD ROBERT RAFTON, OF ANDOVER, MASSACHUSETTS, ASSIGNOR TO RAFFOLD PROCESS CORPORATION, A CORPORATION OF MASSACHUSETTS

## PAPER MANUFACTURE

No Drawing.

Application filed April 29, 1931. Serial No. 533,872.

This invention relates to the manufacture of paper filled with alkaline filler.

The principal object of this invention is to improve the running qualities on the paper machine of paper filled with alkaline filler.

An important object is the minimizing of sticking on the paper machine in the manufacture of such paper.

A further object is the minimizing of the sticking of the web to the press rolls of the paper machine in the running of sized paper filled with alkaline filler.

A further object is the production of higher alumina content rosin size precipitates in the manufacture of paper filled with alkaline filler, particularly by the employment of sodium aluminate therein.

Other objects and advantages of this invention will become apparent during the course of the following description.

In my copending application Serial No. 304,171, filed September 5, 1928, now matured into Patent No. 1,803,646, issued May 5, 1931, I describe a method of substantially eliminating foam in the running of unsized papers filled with an alkaline filler, in one modification of which an amount of sodium resinate insufficient to impart a substantial degree of sizing to the paper is added in the beater, precipitated therein with alum, and then the precipitate which has been deteriorated by contact with alkaline filler is restored at the wet end of the paper machine with a further quantity of alum. In my copending application Serial No. 304,174, filed September 5, 1928, now matured into Patent No. 1,803,649, issued May 5, 1931, I describe a similar process wherein sodium resinate is added in the beater, and alum is added for purposes of precipitation at the wet end of the paper machine.

In my copending applications Serial Nos. 304,168 and 304,172, both filed September 5, 1928, now matured respectively into Patents Nos. 1,803,643 and 1,803,647, both issued May 5, 1931, I describe two processes similar to the above except that in these two cases there is present a sufficient amount of size to produce a substantially sized paper.

In the running of substantially unsized

paper according to the methods referred to in the first two cited applications, no difficulty has been experienced in regard to any tendency of the stock to stick on the paper machine. On the other hand in running sized paper according to the methods described in the later referred to applications, a tendency to stick particularly on the top first press roll has been encountered in certain cases, especially where there has been sufficient size present to produce a hard sized paper.

There is always a tendency in papermaking stocks to stick on the press roll, particularly in heavily sized stocks. This difficulty has lead to the adoption of press rolls of various types such as granite, rubber covered, or the like, which are supposed to reduce the tendency of stock to stick thereon to a greater extent than the types previously used. Furthermore it is well known in the paper industry that changes in the freeness of the stock on the paper machine will change the sticking characteristics of the stock. However in certain cases after all the known expedients had been tried, there seemed to be a greater sticking tendency in the stocks run according to the methods disclosed in the two cited applications last referred to above than in clay-filled paper stocks run under similar conditions on the same paper machines.

In the course of an investigation conducted to determine the cause of this sticking, it was observed that the pH values of the stocks on the wires of the paper machines in the cases where my said methods were practiced were usually higher than in the cases where stocks containing no filler or containing inert filler such as clay were being run. As a result of this observation, the composition of rosin size precipitates prepared at different pH values was determined, i. e. to a series of samples of diluted rosin size were added respectively the amounts of alum necessary to produce successively lower pH values. It was found that the precipitates produced at the higher pH values were very sticky and difficult to filter, this being particularly the case at pH values higher than 7, whereas the precipitates produced at pH values of 7 or lower were sub-

stantially non-sticky, and filtered relatively easily.

An analysis of the precipitates produced as above showed that the alumina content of the precipitates varied according to the pH at which the precipitate had been produced, the amount of alumina increasing with decrease in pH. The increase was very marked in an experiment, in the first part of which 10 a sample of rosin size was precipitated with an amount of alum previously found to give a definite pH, in this instance 8.5, at which pH the precipitation of the rosin size was not complete. The precipitate was then filtered off, further alum added to the filtrate, and a further filtration made. By repeating this process, a series of precipitates was obtained, made from solutions of rosin size of successively lesser pH values and precipitated with 15 amounts of alum which gave still lower definite pH values. As stated, the alumina content of this series of precipitates rose rapidly with decrease in the final pH. It therefore appeared that in view of the difficulty of 20 maintaining a very low pH on the paper machine in the presence of alkaline filler, if it were possible to increase the alumina content of the size precipitate, that the sticking qualities of the such size precipitate might 25 be markedly altered.

After considerable experimentation it was found that by a special procedure alumina could be introduced into a size precipitate at any given pH in quantities much greater than 30 would normally be introduced at that pH were the size merely precipitated at that pH with alum. This was accomplished by mixing the size, prior to its precipitation with alum, with a compound of aluminum which did not cause its precipitation, preferably a non-acid compound of aluminum, preferably in soluble form. A suitable compound of aluminum for carrying out this procedure was found to 35 be sodium aluminate. Sodium aluminate was 40 mixed with size prior to the precipitation thereof, and then precipitation with an acidic material such as alum was effected at a high pH value such as 8. When precipitation of other similar samples was effected at successively lower pH values and it was found that 45 the alumina content of the thus produced precipitates was greatly increased over those produced at similar pH values where no sodium aluminate had been admixed with the size. 50 In effect it was found that precipitates produced from rosin size at relatively high pH values could be made with as great or even a much greater alumina content than those produced with alum alone at a relatively low pH. The precipitates so produced with a high content of alumina even at a relatively high pH were found to be substantially less sticky, than the similar low alumina precipitates made at the same pH. Likewise the high alumina content precipitates produced at 55 60 65

lower pH values were also found to be substantially non-sticky. It is thus seen that by utilizing this data it is possible to produce rosin size precipitates in practical operation which are substantially non-sticky even though the pH at which they are precipitated may be high and/or the pH of the stock on the wire may be neutral or even higher, due to the presence of alkaline filler. 70

Instead of employing sodium aluminate or 75 other alkaline aluminate with the size I may actually prepare the size by original solution of the rosin with sodium aluminate, or with sodium aluminate in conjunction with other alkalies. This is a convenient method as by 80 so doing one less constituent has to be handled, and also part of the alkalinity of the sodium aluminate is used up in the solution of the rosin during the preparation of the size and hence the subsequent quantity of 85 acidic material required for precipitation is materially reduced.

Instead of using sodium aluminate or other alkaline aluminate I have found that it is possible to prepare a solution of an aluminum compound at a pH value at which aluminum hydroxide or hydrate would ordinarily be precipitated, by having present a precipitation inhibitor such for example as a citrate, either citric acid, or a soluble citrate such as 90 sodium, potassium or ammonium citrate, being suitable. In such case a solution of sodium citrate for example may be added to alum and sufficient alkali, such as sodium carbonate for example, may be added to raise the pH 95 of the alum to neutrality or even higher without the precipitation of alumina taking place. When such a neutralized or alkalinized substantially non-precipitating aluminum solution is prepared and added to rosin size, and then the rosin size precipitated in the presence thereof by the addition of an acidic material such as alum, the precipitate thus obtained is substantially non-sticking. There has not as yet, however, been sufficient analytical data adduced to prove conclusively 100 that the rosin size precipitates so obtained have a higher alumina content than a normal rosin size precipitate, but from the trend of data so far obtained such a conclusion seems 105 110 to be probable. Instead of citric acid or citrates as precipitation inhibitors, other materials may be used such for example as tartrates, but the citrates seem to be most effective materials yet tried. Aluminum citrate itself may also be used directly, instead of mixing a compound of aluminum and a citrate. 115 120 125

I am aware of the fact that it has previously been known to use sodium aluminate in connection with rosin size in the beater, and also to dissolve rosin size with sodium aluminate, and precipitate such sizes in the beater. However any such size precipitates, or precipitates made by the citrate method as indicated 130

above, if produced in the ordinary way in the beater and subjected to the action therein of alkaline filler, would be speedily deteriorated, even to the point of complete destruction and 5 would thus be of no commercial use. It is only by employing my new technique (explained below) of adding materials in the manufacture of paper filled with alkaline filler under conditions favoring the minimizing 10 of the time and/or intimacy of contact of the constituents of the mix, that the facts adduced herein become capable of utilization.

In the preferred practice of my invention size such as rosin size is added to fibrous material in a beater. An aluminate such as sodium aluminate should be present, and it is suitably added mixed with the size; or instead of the aluminate being present independently, the rosin size used may be made 20 with sodium aluminate. The size is precipitated in the beater with an acidic material such as alum, in which case if, due to the presence of alkaline filler in the stock in the beater, the size precipitate is deteriorated, it is restored, preferably with a further quantity of 25 alum, by the addition thereof under conditions favoring the minimizing of the time and/or intimacy of contact of the constituents of the mix, for example at the wet end of the paper machine. Or the size may be originally precipitated by the alum added at the wet end of the paper machine, or both the size and the alum may be added at the wet end of the 30 paper machine, or the size may be added at that point to a stock to which alum has previously been added. In the latter case of course the aluminate must accompany the size when added. The alkaline filler may be added in the beater or at the wet end of the 35 paper machine, as described in various of my copending applications in which it is disclosed that alkaline filler and/or alum may be added to the fibrous mix at the wet end of the paper machine. In addition to my co- 40 pending applications already noted, reference is made to my applications Serial Nos. 304,167 and 304,175, both filed September 5, 1928, and No. 321,754 filed November 24, 1928, now matured respectively into Patents Nos. 50 1,803,642 and 1,803,650, both issued May 5, 1931, and 1,808,071, issued June 2, 1931. The various possibilities of the precipitation of size in papers filled with alkaline fillers have been thoroughly discussed in my said prior 55 applications, but according to the improvement described herein it is necessary that the precipitation of the size must take place in the presence of a substantially non-acid aluminum compound in order to obtain the desired beneficial substantially non-sticking 60 characteristic of the resulting size precipitate.

While I do not limit myself to the use of any definite quantities of sodium aluminate in the practice of my invention, I have found 65 that a very satisfactory amount to employ is

an amount of aluminate which represents 10-15% of alumina calculated as  $Al_2O_3$  based on the amount of dry rosin in the rosin size used. A quantity of alum for precipitation of the size is then used which would be at 70 least sufficient, but preferably in some excess over that quantity required, to give a neutral or slightly acid reaction with said amount of size and said amount of aluminate. It is not possible to give in general the quantity 75 of alum required owing to the great variability in the amount of alkali present in sodium aluminates, but the minimum quantity required can be easily determined in the laboratory by a simple stoichiometrical titration. From the above it will be apparent that other things being equal it is desirable to use the sodium aluminate as weakly alkaline as possible.

With respect to the amount of precipitation inhibitor suitably to be present when this modification of my invention is to be employed, while I do not limit myself thereto, I have found that an amount of sodium citrate equal to approximately 50% calculated as weight of dry commercial citrate on the weight of dry alum which is neutralized or alkalinized is a suitable quantity to employ. The neutralized or alkalinized alum to be used may suitably be approximately 75% dry 85 alum based on weight of dry size employed.

Cross reference is here made to my copending applications Serial Nos. 319,719, 319,720 and 319,721, all filed November 15, 1928, now matured respectively into Patents Nos. 1,808,067, 1,808,068 and 1,808,069, all issued 100 June 2, 1931, wherein there is described methods of incorporating into a paper an inorganic alkali metal salt with a pH value greater than 7.0, which is precipitable by material which depresses its hydroxyl ion concentration. It will be noted that sodium aluminate is such a compound but no claims 105 specifically to sodium aluminate are made therein.

In my various copending applications referred to herein as well as in others, I have discussed in full the principle on which the expression "minimizing the time and/or intimacy of contact of the constituents of the mix" is based. Briefly it is that alkaline filler, which always is present in the stock from which paper filled with alkaline filler is made in great stoichiometrical excess over the acidic constituent, acts upon the acidic constituent to the ultimate destruction thereof and/or the destruction of the effect maintained by such constituent. (The acidic constituent so-called may be one which is actually acid, and/or one which such as a size precipitate is capable of being affected or deteriorated by an alkaline material). The action just referred to has been found to depend upon the time of contact of the acidic and 115 alkaline constituents and also upon the in- 120 125 130

timacy of contact of these constituents. Agitation such as normally occurs in papermaking procedure in stuff chests or the like accelerates the rate of reaction, but agitation at low concentrations while having some effect is not nearly so deleterious. Based on this principle a practical application has been developed whereby, by minimizing the time and/or intimacy of contact of the acidic and 10 alkaline constituents, the acidic constituent and/or the effect produced thereby, is substantially preserved in an alkaline filler mix. With the present types of paper machines and the present arrangement of apparatus 15 usually employed in paper machine operation, the contact of the acidic material and the alkaline constituent at any time prior to the passage of the stock from the last stuff chest, which is commonly called the "ma- 20 chine chest", results in great deterioration of complete destruction of the acidic material. Addition of one or both of these constituents, as well as other materials such as size, sodium silicate, starch and the like as set forth in my 25 various copending applications, at a point subsequent to the passage of the stock from the machine chest, after which point according to present day operating practice the stock remains in concentrated condition only 30 for a very brief interval of time or addition preferably at or subsequent to the point of dilution, i. e. at the wet end of the paper machine, serves to substantially conserve the acidic material and/or effect thereof in the 35 fibrous mix. It is the application of this principle which I utilize in connection with the precipitation of rosin size in the presence of substantially non-acid aluminum compound as set forth in the description of the 40 preferred practice of my invention given above.

I have also found that the introduction of sodium aluminate is at times desirable in the manufacture of substantially unsized 45 paper filled with alkaline filler, and that it may be incorporated into such paper in general according to the methods herein discussed even in the absence of rosin size or in the presence of an amount of rosin size in- 50 sufficient to impart a substantial degree of sizing to the resulting paper. The use of sodium aluminate or of a non-acid aluminum compound whose solubility is maintained by the presence of a precipitation inhibitor pre- 55 sents a means for introducing into a paper mix an acidic aluminum compound without the direct addition thereto of such com- 60 pound, when an acidic condition is also present in the paper mix, or when an acidic material is added thereto, which can react with the non-acid aluminum compound to produce an acidic aluminum compound.

In the practice of my invention instead of sodium aluminate or of a substantially non- 65 acid aluminum compound whose precipita-

tion is inhibited by the action of a precipitation inhibitor, I may employ as equivalents with a measure of success similar compounds of other metals such as tin, zinc, and the like, but from the experiments so far conducted 70 I find that the aluminum compounds are the most efficient as well as the most inexpensive.

For size I may use rosin size, or any size which may be used as a substitute therefor in the paper industry, such as saponified 75 fatty acids or the like.

For precipitant or restoring agent, or for use with the non-acid compound of aluminum in substantially unsized papers, I may use alone or in combination acidic materials, 80 such as a mineral or other acids, particularly metallic salts such as compounds of aluminum, zinc, tin, or the like.

The term "paper mix" as used herein is intended to mean a mix of various constituents including fibre from which paper may be made, either alone or after the addition of other ingredients.

By the term "alkaline filler" I mean substantially water insoluble filler which when 90 agitated in contact with freshly boiled distilled water, say for an hour, will impart a pH value to such water greater than 7.0, that is, which will be on the alkaline side of the neutral point. Among fillers included 95 in this group may be mentioned calcium carbonate, of which lime mud from the causticizing process is one form; calcium carbonate magnesium basic carbonate employed in the paper disclosed in my U. S. Patent No. 100 1,595,416 of August 10, 1926; calcium carbonate magnesium hydroxide disclosed in my U. S. Patent No. 1,415,391 of May 9, 1922; and other substantially water insoluble normal or basic carbonates of alkaline earth 105 metals, (which expression is herein intended to include magnesium), or compounds, double salts, or physically associated mixtures of these with one or more other acid soluble materials of a substantially water insoluble 110 nature.

Where I speak of sizing, paper, or the like, as containing "alumina", I do not mean to restrict myself to the presence of any definite compound of aluminum therein, but rather I use the term in its ordinarily accepted meaning to indicate that a compound of aluminum is present, the aluminum content of which may be determined by analytical procedure as alumina ( $Al_2O_3$ ). 120

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine. 125

By the term "wet end of the paper ma- 130

chine", I intend to include those instrumentalities employed in paper manufacture by which and/or in which a relatively concentrated paper mix is diluted, and treated, conveyed or fed up to the point of web-formation, such as the mixing box, regulating and proportioning devices, riffles, troughs, screens, head boxes, inlets and the like, including also instrumentalities used in the white water cycle.

It is to be understood that my invention is not dependent upon or limited by any theory expressed herein; and as no one theory of the mechanism of sizing has as yet found general acceptance in the art, some theories holding that the alumina is integral with the sizing and some that it is merely jointly present therewith, it is to be understood that where I speak of a size precipitate or sizing as containing alumina I mean that such alumina may literally be integral therewith or that it may be jointly present therewith in the fibrous mix or paper in question.

While I have described in detail the preferred embodiments of my invention, it is to be understood that the details of procedure, the proportions of ingredients, and the arrangement of steps may be widely varied without departing from the spirit of my invention or the scope of the subjoined claims.

I claim:

1. In a method of manufacturing paper filled with alkaline filler wherein material is added to a paper mix under conditions favoring the minimizing of the time and/or intimacy of contact of the constituents of the mix, the step of adding to said mix a non-acid aluminum compound.

2. In a method of manufacturing paper filled with alkaline filler wherein material is added to a paper mix under conditions favoring the minimizing of the time and/or intimacy of contact of the constituents of the mix, the step of adding to said mix a non-acid aluminum compound in soluble condition.

3. In a method of manufacturing paper filled with alkaline filler wherein material is added to a paper mix under conditions favoring the minimizing of the time and/or intimacy of contact of the constituents of the mix, the step of adding to said mix a soluble non-acid aluminum compound precipitable by acidic material.

4. In a method of manufacturing paper filled with alkaline filler wherein material is added to a paper mix under conditions favoring the minimizing of the time and/or intimacy of contact of the constituents of the mix, the steps of adding to said mix a soluble non-acid aluminum compound precipitable by acidic material, and acidic material.

5. In a method of manufacturing paper filled with alkaline filler wherein material is added to a paper mix under conditions favor-

ing the minimizing of the time and/or intimacy of contact of the constituents of the mix, the steps of adding to said mix a soluble non-acid aluminum compound precipitable by metallic salt, and a metallic salt.

6. In a method of manufacturing paper filled with alkaline filler wherein material is added to a paper mix under conditions favoring the minimizing of the time and/or intimacy of contact of the constituents of the mix, the steps of adding to said mix a soluble non-acid aluminum compound precipitable by alum, and alum.

7. In a method of manufacturing paper filled with alkaline filler wherein material is added to a paper mix under conditions favoring the minimizing of the time and/or intimacy of contact of the constituents of the mix, the step of adding to said mix a non-acid aluminum compound soluble due to the presence of a precipitation inhibitor.

8. In a method of manufacturing paper filled with alkaline filler wherein material is added to a paper mix under conditions favoring the minimizing of the time and/or intimacy of contact of the constituents of the mix, the step of adding to said mix a non-acid aluminum compound soluble due to the presence of a precipitation inhibitor, said inhibitor comprising a citrate radicle.

9. In a method of manufacturing paper filled with alkaline filler wherein material is added to a paper mix under conditions favoring the minimizing of the time and/or intimacy of contact of the constituents of the mix, the steps of adding to said mix a non-acid aluminum compound soluble due to the presence of a precipitation inhibitor, and acidic material.

10. In a method of manufacturing paper filled with alkaline filler wherein material is added to a paper mix under conditions favoring the minimizing of the time and/or intimacy of contact of the constituents of the mix, the step of adding to said mix sodium aluminate.

11. In a method of manufacturing paper filled with alkaline filler wherein material is added to a paper mix under conditions favoring the minimizing of the time and/or intimacy of contact of the constituents of the mix, the steps of adding to said mix sodium aluminate and acidic material.

12. In a method of manufacturing paper filled with alkaline filler wherein material is added to a paper mix under conditions favoring the minimizing of the time and/or intimacy of contact of the constituents of the mix, the steps of adding to said mix sodium aluminate and alum.

13. In a method of manufacturing paper filled with alkaline filler wherein material is added to a paper mix under conditions favoring the minimizing of the time and/or intimacy of contact of the constituents of the

- mix, the step of precipitating size in the presence of a non-acid compound of aluminum.
14. In a method of manufacturing paper filled with alkaline filler wherein material is added to a paper mix under conditions favoring the minimizing of the time and/or intimacy of contact of the constituents of the mix, the step of precipitating size in the presence of a non-acid compound of aluminum in soluble condition. 70
15. In a method of manufacturing paper filled with alkaline filler wherein material is added to a paper mix under conditions favoring the minimizing of the time and/or intimacy of contact of the constituents of the mix, the step of precipitating size in the presence of a non-acid compound of aluminum soluble due to the presence of a precipitation inhibitor. 75
16. In a method of manufacturing paper filled with alkaline filler wherein material is added to a paper mix under conditions favoring the minimizing of the time and/or intimacy of contact of the constituents of the mix, the step of precipitating size in the presence of a non-acid compound of aluminum soluble due to the presence of a precipitation inhibitor, said inhibitor comprising a citrate radicle. 80
17. In a method of manufacturing paper filled with alkaline filler wherein material is added to a paper mix under conditions favoring the minimizing of the time and/or intimacy of contact of the constituents of the mix, the step of precipitating size with acidic material in the presence of a non-acid compound of aluminum in soluble condition. 85
18. In a method of manufacturing paper filled with alkaline filler wherein material is added to a paper mix under conditions favoring the minimizing of the time and/or intimacy of contact of the constituents of the mix, the step of precipitating size with metallic salt in the presence of a non-acid compound of aluminum in soluble condition. 90
19. In a method of manufacturing paper filled with alkaline filler wherein material is added to a paper mix under conditions favoring the minimizing of the time and/or intimacy of contact of the constituents of the mix, the step of precipitating size with alum in the presence of a non-acid compound of aluminum in soluble condition. 95
20. In a method of manufacturing paper filled with alkaline filler wherein material is added to a paper mix under conditions favoring the minimizing of the time and/or intimacy of contact of the constituents of the mix, the step of precipitating size in the presence of sodium aluminate. 100
21. In a method of manufacturing paper filled with alkaline filler wherein material is added to a paper mix under conditions favoring the minimizing of the time and/or intimacy of contact of the constituents of the mix, the step of precipitating size with acidic material in the presence of sodium aluminate. 105
22. In a method of manufacturing paper filled with alkaline filler wherein material is added to a paper mix under conditions favoring the minimizing of the time and/or intimacy of contact of the constituents of the mix, the step of precipitating size with alum in the presence of sodium aluminate. 110
23. In a method of manufacturing paper filled with alkaline filler wherein material is added to a paper mix under conditions favoring the minimizing of the time and/or intimacy of contact of the constituents of the mix, the step of precipitating rosin size in the presence of a non-acid compound of alum. 115
24. In a method of manufacturing paper filled with alkaline filler wherein material is added to a paper mix under conditions favoring the minimizing of the time and/or intimacy of contact of the constituents of the mix, the step of precipitating rosin size in the presence of a non-acid compound of aluminum in soluble condition. 120
25. In a method of manufacturing paper filled with alkaline filler wherein material is added to a paper mix under conditions favoring the minimizing of the time and/or intimacy of contact of the constituents of the mix, the step of precipitating rosin size in the presence of sodium aluminate. 125
26. In the manufacture of paper filled with alkaline filler the step comprising the addition to the paper mix of an inorganic alkali metal salt with a pH value greater than 7.0, which is precipitable by material which depresses its hydroxyl ion concentration, under conditions favoring the minimizing of the time of contact of the constituents of the mix. 130
27. In the manufacture of paper filled with alkaline filler the step comprising the addition to the paper mix of an inorganic alkali metal salt with a pH value greater than 7.0, which is precipitable by material which depresses its hydroxyl ion concentration, under conditions favoring the minimizing of the time and intimacy of contact of the constituents of the mix. 135
28. In the manufacture of paper filled with alkaline filler the step comprising the addition to the paper mix at the wet end of the paper machine of an inorganic alkali metal salt with a pH value greater than 7.0, which is precipitable by material which depresses its hydroxyl ion concentration. 140
29. In the manufacture of paper filled with alkaline filler the step comprising the addition to the paper mix of an inorganic alkali metal salt with a pH value greater than 7.0, which is precipitable by material which depresses its hydroxyl ion concentration, and a precipitant therefor, under conditions favoring the minimizing of the time of contact of the constituents of the mix. 145

30. In the manufacture of paper filled with alkaline filler the step comprising the addition to the paper mix of an inorganic alkali metal salt with a pH value greater than 7.0, which  
 5 is precipitable by material which depresses its hydroxyl ion concentration, and a precipitant therefor, under conditions favoring the minimizing of the time and intimacy of contact of the constituents of the mix. 70
- 10 31. In the manufacturing of paper filled with alkaline filler the step comprising the addition to the paper mix at the wet end of the paper machine of an inorganic alkali metal salt with a pH value greater than 7.0, which  
 15 is precipitable by material which depresses its hydroxyl ion concentration, and a precipitant therefor. 75
- 20 32. In the manufacture of paper filled with alkaline filler, the step which comprises providing in the fibrous mix a size precipitate containing alumina derived at least in part from a substantially soluble non-acid compound of aluminum. 80
- 25 33. In the manufacture of paper filled with alkaline filler comprising calcium carbonate, the step which comprises providing in the fibrous mix a size precipitate containing alumina derived at least in part from sodium aluminate. 85
- 30 34. In the manufacture of paper filled with alkaline filler, the step comprising the addition to the fibrous mix of substantially soluble non-acid aluminum compound. 90
- 35 35. In the manufacture of paper filled with alkaline filler comprising calcium carbonate, the improvement comprising the addition to the fibrous mix of size and substantially soluble non-acid aluminum compound. 95
- 40 36. In the manufacture of paper filled with alkaline filler comprising calcium carbonate, the step comprising the addition to the fibrous mix of sodium aluminate. 100
- 45 37. In the manufacture of paper filled with alkaline filler the step comprising the addition to the fibrous mix of an inorganic alkali metal salt with a pH value greater than 7.0 which is precipitable by depression of its hydroxyl ion concentration. 110
- 50 38. In the manufacture of paper filled with alkaline filler comprising calcium carbonate, the improvement comprising the addition to the fibrous mix of size and an inorganic alkali metal salt with a pH value greater than 7.0 which is precipitable by depression of its hydroxyl ion concentration. 115
- 55 39. Filled paper comprising fibrous material, alkaline filler, and alumina derived from substantially soluble non-acid compound of 120  
 60 pound of aluminum. 125
- 65 40. Filled paper comprising fibrous material, alkaline filler comprising calcium carbonate, and alumina derived from substantially soluble non-acid compound of 130  
 65 aluminum.